

## UNITED STATES PATENT OFFICE

2,261,985

## FIBROUS TUBE

Albert E. Forster, Wilmington, Del., assignor to  
 Hercules Powder Company, Wilmington, Del.,  
 a corporation of Delaware

No Drawing. Application January 11, 1940,  
 Serial No. 313,377

6 Claims. (CL. 138—76)

This invention relates to fibrous tubes and more particularly to impregnated fibrous tubes suitable for use as temporary bore hole casings and as pipes for fluids.

An object of the present invention is to provide inexpensive impregnated fibrous tubes which are light in weight and are relatively strong and rigid.

Another object is to provide impregnated fibrous tubes which resist moisture for a period of time and then are adapted to become saturated and deteriorate.

A further object is to impregnate fibrous tubes with a temporary moisture-proofing composition which is readily adsorbed by the fibers of the tubes.

Other and further objects will be obvious upon an understanding of the illustrative embodiment about to be described, or will be indicated in the appended claims, and various advantages not referred to herein will occur to one skilled in the art upon employment of the invention in practice.

These objects, generally, are accomplished by impregnating tubes formed of paper, cardboard, pulp board, or similar cellulosic fibrous materials, preferably having a thickness of between .1 and .2 of an inch, and a diameter of about 3 inches. The impregnating composition, which produces the foregoing desired results, may consist of a substantially petroleum-hydrocarbon insoluble pine wood resin, or may comprise a mixture of the resin and bituminous or asphaltic material, such as coal tar, or, if desired, the composition may comprise a plastic-like reaction product of the resin and an oil, and bituminous or asphaltic material. Also, if desired, a mixture of the reaction product and the coal tar may be employed.

The material which is characterized by the term "substantially petroleum-hydrocarbon insoluble pine wood resin," herein and in the appended claims, is the resinous material which may be prepared from pine wood, preferably from stump pine wood, in the following manner. The pine wood, which may or may not have been steamed to remove volatile constituents such as turpentine and pine oil, may be extracted with a coal tar hydrocarbon such as benzol or toluol, and the extract then freed of volatile constituents, leaving a residue consisting of a mixture of wood rosin and the resin used in the present compositions. Extraction of this mixture with a petroleum hydrocarbon such as, for example, gasoline, dissolves and removes

the rosin. After separation of the rosin, high in abietic acid, a resinous residue remains which is low in abietic acid.

Alternatively, a gasoline solution of the residue from the initial coal tar hydrocarbon extract may be treated with furfural, and the two layers which form separated, in which case the petroleum-hydrocarbon insoluble pine wood resin is found dissolved in the furfural from which it may be obtained by evaporation of the furfural.

Another method of producing the resin comprises extracting resin from the wood by means of benzol and treating the extracted resin with a mixture of gasoline and furfural. The gasoline dissolves the rosin while the furfural dissolves the resin. The solvents are then separated and the resin is recovered by evaporation of the furfural.

This resinous material, used in carrying out the present invention, is characterized by a dark red brown color, cherry red in solution, and by substantial insolubility in petroleum hydrocarbons, but it will vary somewhat in its specific characteristics such as acid number, melting point, exact petroleum ether solubility, and content of naphtha and toluol insoluble material, depending upon the details of the extraction process utilized. This resin will meet or nearly meet the following specifications, namely, substantial insolubility in petroleum hydrocarbons, substantially complete solubility in alcohol, a methoxy content from about 3% to about 7.5% (usually from about 4% to about 6%), an acid number in the range from about 90 to about 110, and a drop melting point in the range from about 95° C. to about 125° C.

The coal tar which is suitable in the composition may be a high boiling coal tar oil or a coal tar pitch.

The oil used in making the plastic-like reaction product may be a semi-drying oil, such as fish oil or a drying oil, such as linseed oil, which preferably can be cooked to compatibility with the resin. Where "fish oil" is mentioned hereinafter and in the claims, it is intended to include such semi-drying or drying oils generally known. If desired, in preparing the reaction product, hexamethylenetetramine or formaldehyde is added to assist the partial conversion of the resin to a gel.

The present invention is not intended to be limited to specific proportions of ingredients. It has been found that an impregnating composition consisting only of the substantially petroleum hydrocarbon insoluble pine wood resin is

suitable. This resin may be modified with coal tar. For example, for every ten parts of coal tar between about 1 part and about 90 parts resin may be used. Where the reaction product of the resin with a drying or semi-drying oil is added to about 10 parts coal tar, up to about 40 parts resin, and between 10 and 200 parts reaction product comprise the composition. The reaction product may vary in composition, between about 33% and 70% resin and the balance drying or semi-drying oil to total 100%. A small amount of hexamethylenetetramine or formaldehyde is added to facilitate conversion of the resin.

The following examples illustrate compositions suitable for impregnating fibrous cellulosic tubes to accomplish the objects of the present invention:

*Materials (parts by weight)*

|                     | Examples |    |     |    |     |    |
|---------------------|----------|----|-----|----|-----|----|
|                     | I        | II | III | IV | V   | VI |
| Resin*              | 100      | 90 | 40  | 40 | 10  | 10 |
| Coal tar oil        |          | 10 | 10  | 10 | 10  | 90 |
| Coal tar pitch      |          |    |     |    |     |    |
| Reaction product GF |          |    | 10  |    | 10  |    |
| Reaction product FF |          |    |     |    | 200 |    |
| Reaction product AF |          |    |     |    |     |    |

\*Substantially petroleum hydrocarbon insoluble pine wood resin. GF, a fish oil plastic, 33% "resin," partly converted to a gel with hexamethylenetetramine. FF, 50% "resin" with fish oil cooked to convertibility with formaldehyde. AF, 70% "resin" with fish oil cooked to compatibility.

The impregnating compositions may be prepared by heating the materials to provide a low melt having a viscosity to facilitate penetration of the fibrous tubes. Preferably, the impregnation of the tubes is carried out in a vessel maintained under a pressure of about 70 pounds per square inch, by the addition of an inert gas, such as nitrogen, while maintaining the temperature of the melt between about 120° and 180° C., but preferably at about 165° C. By impregnating under pressure, the cellulosic fibers are not degraded by the heat of the melt. The tubes thereafter may be removed from the impregnating bath and permitted to drain and dry in a suitable manner.

If desired, the tubes may be coated, impregnated, or saturated by brushing, coating or spraying the compositions thereon or dipping the tubes therein. The amount of material absorbed may be controlled to provide the tubes with any desired degree of water resistance.

The tubes impregnated in the foregoing manner by using the compositions described herein are suitable where a semi-permanent or temporary tubing is desired. For example, where temporary pipe lines for pumping water are desired at locations such as swamp or marsh land, which

are not readily accessible by motor trucks, the tubes, by being light in weight, can be readily carried manually. After the pipe lines are no longer desired, the tubes need not be recovered as would be the case of more expensive metal pipe, but can be left at the location and upon being exposed to rain and sun will deteriorate.

The tubes, in accordance with the invention, are also suitable for lining bore holes used for explosive charges in seismic prospecting. Here again the tubes are readily brought on location, are sufficiently strong to keep the bore hole open to permit the desired number of charges to be exploded and can thereafter be abandoned and permitted to deteriorate without becoming a menace to tilling of the soil, or to navigation in the event they are used for lining holes beneath the surface of lakes or bays.

The tubes so impregnated may be of any suitable design. For example, tubes formed of spirally wound strips may be used. The impregnating composition serves to strengthen the joints of the strips and serves to prevent unravelling thereof.

It will be understood that the details and examples hereinbefore set forth are illustrative only and that the invention as broadly described and claimed is in no way limited thereby.

What I claim and desire to protect by Letters Patent is:

1. A tube of the class described composed of fibrous cellulosic material impregnated with a material selected from the group consisting of a substantially petroleum-hydrocarbon insoluble pine wood resin, and reaction products of said resin with a semi-drying oil.

2. A tube of the class described composed of fibrous cellulosic material impregnated with a mixture comprising coal tar and a material selected from the group consisting of a substantially petroleum-hydrocarbon insoluble pine wood resin, and reaction products of said resin with a semi-drying oil.

3. A tube of the class described composed of fibrous cellulosic material impregnated with a substantially petroleum hydrocarbon insoluble pine wood resin.

4. A tube of the class described composed of fibrous cellulosic material impregnated with a mixture consisting of coal tar and a substantially petroleum-hydrocarbon insoluble pine wood resin.

5. A tube of the class described composed of fibrous cellulosic material impregnated with a mixture comprising coal tar, and a reaction product of a fish oil and a substantially petroleum-hydrocarbon insoluble pine wood resin.

6. A tube of the class described composed of fibrous cellulosic material impregnated with a mixture consisting of a coal tar, a substantially petroleum-hydrocarbon insoluble pine wood resin, and a reaction product of said resin and a fish oil.

ALBERT E. FORSTER.

## DISCLAIMER

2,261,985.—*Albert E. Forster*, Wilmington, Del. FIBROUS TUBE. Patent dated November 11, 1941. Disclaimer filed May 11, 1943, by the assignee, *Hercules Powder Company*.

Hereby enters this disclaimer to as much of claim 1 as will include a substantially petroleum-hydrocarbon insoluble pine wood resin as the impregnating material; and to claim 3 in said patent.

[*Official Gazette June 1, 1943.*]